# EUROPEAN PATENT APPLICATION

(11) **EP 1 186 679 A1**
(43) Date of publication of application: **13.03.2002**
(21) Application number: 00203141.7
(22) Date of filing: 12.09.2000
(51) Int. Cl.: C23C 2/06

(54) **Hot-dip galvanising alloy and process**

(71) Applicant: n.v. Umicore s.a., 1000 Bruxelles (BE)
(72) Inventor: Gilles, Mik, c/o N.V. Union Miniere S.A., 2250 Olen (BE)
(74) Representative: Saelemaekers, Juul

(57) **Abstract**

Alloy and process for galvanising steel by immersion in a zinc alloy containing bath comprising by weight 0.1 to less than 1% Bi, 0.01 to 0.05% Al, 0.04 to 0.12% Ni up to 0.05% Mn, the rest being zinc and unavoidable impurities.

## Description

The present invention relates to a bath for hot-dip galvanising consisting of alloyed zinc, that is particularly useful for batchwise galvanising steel articles.

Conventional galvanisation practice results in a coating thickness of 70 to 120 µm. A drawback of such thick coatings is the reduced resistance to stress induced crack formation.

The aim of the present invention is therefore to provide a bath composition for hot-dip galvanising, which results in a coating thickness of 30 to 50 µm. Also, the thickness of the intermetallic layer is reduced to approximately 30 to 35 µm. This induces an increased resistance to stress induced crack formation as required e.g. for critical parts in the automotive industry.

According to the invention the bath contains, by weight, 0.1 to less than 1 % Bi, 0.01 to 0.05 % Al, 0.04 to 0.12 % Ni, up to 0.05 % Mn, the rest being zinc and unavoidable impurities. Preferably, the bath contains 0.3 to 0.8 % Bi, 0.02 to 0.04 % Al, 0.06 to 0.10 % Ni and up to 0.05 % Mn. A bath composition with 0.5 % Bi, 0.03 % Al and 0.08 % Ni is especially preferred.

The galvanising process using the alloy of the invention is particularly suitable for coating low reactivity steel. By low reactivity steel is meant steel comprising, by weight, Si and P in such amounts that Si < 0.03 % and % Si + 2.5 x % P < 0.09.

## Claims

1. An alloy for hot-dip galvanising steel comprising, by weight, 0.1 to less than 1 % Bi, 0.01 to 0.05 % Al, 0.04 to 0.12 % Ni, up to 0.05 % Mn, the rest being zinc and unavoidable impurities.

2. An alloy according to claim 1, comprising, by weight, 0.3 to 0.8 % Bi, 0.02 to 0.04 % Al, 0.06 to 0.10 % Ni, up to 0.05 % Mn, the rest being zinc and unavoidable impurities.

3. A process for galvanising steel by immersion in a zinc alloy galvanising bath comprising the step of immersing the steel articles in a molten bath of a zinc alloy comprising, by weight, 0.1 to less than 1 % Bi, 0.01 to 0.05 % Al, 0.04 to 0.12 % Ni, up to 0.05 % Mn, the rest being zinc and unavoidable impurities.

4. A process according to claim 3, **characterised in that** the steel articles comprise, by weight, Si and P in such amounts that Si < 0.03 % and % Si + 2.5 x % P < 0.09.
